

## UNITED STATES PATENT OFFICE

2,436,347

## GREASE COMPOSITIONS

John C. Zimmer, Union, and Arnold J. Morway,  
 Clark Township, Union County, N. J., assignors  
 to Standard Oil Development Company, a cor-  
 poration of Delaware

No Drawing. Application December 30, 1944,  
 Serial No. 570,784

9 Claims. (Cl. 252—36)

1

The present invention relates to the field of greases, and more particularly to improvements in low temperature greases. In the usual methods of manufacturing low temperature greases, low boiling mineral oil fractions with resultant low flash points and low viscosities are compounded with metallic soaps to form plastic masses, or semi-solid grease compositions. It has been observed that the torque necessary to turn a bearing lubricated by grease is directly proportional to the viscosity of the oil used in the grease at the particular temperature. Therefore it has been necessary in the manufacture of low temperature greases to use low boiling mineral oil fractions since these fractions have low viscosities at extremely low temperatures ( $-100^{\circ}$  F.). However, since the equipment, for instance the shutter on an aerial reconnaissance camera, on which this grease is to be used may at times be subjected to relatively high temperatures ( $150^{\circ}$  F.), the low boiling fractions used in making the grease are limited to those which are not too volatile. The use of extremely low boiling mineral oil fractions in the manufacture of low temperature greases is therefore subject to drastic restrictions because of the high volatility of such fractions and also their use creates operational difficulties during manufacture in the nature of fire hazards. Also after the lubricant has been subjected to high temperatures, loss by volatility may result in a product which is deficient in low temperature characteristics when again used at low temperature if not relubricated.

It has now been found that the esters of aliphatic dibasic acids, particularly those esters in which the esterifying radical is a branched chain alkyl radical, may be substituted for low boiling mineral oil fractions in the production of low temperature greases. These esters possess unusually high boiling points and resulting low vapor pressures at ambient temperatures, high viscosity indices, or low viscosity-temperature coefficient, extremely low pour points and are relatively stable chemically. Among the aliphatic dicarboxylic acids suitable for the preparation of the esters used in making the grease compositions of the present invention there may be mentioned malonic, succinic, isosuccinic, glutaric, ethyl malonic, pyro tartaric, adipic, pimelic, suberic, azelaic and sebatic acids. Instead of one of the enumerated acids, any acid or mixture of acids having the formula  $\text{HOOC}(\text{R})\text{COOH}$ , where R is a bivalent aliphatic hydrocarbon radical—for example synthetic acids produced by polymerization or dimerization of unsaturated fatty

acids or their esters—may be used. The esters which may be used in making the grease compositions of the present invention have the general formula  $\text{COOR}_1-\text{R}-\text{COOR}_2$ , where R is a bivalent aliphatic hydrocarbon radical such as methylene, polymethylene, ethylidene, propylidene, methyl dimethylene, butenylidene and the like; R<sub>1</sub> and R<sub>2</sub> are hydrocarbon radicals such as branched chain alkyl, alkaryl and cyclo alkyl radicals of which secondary butyl, benzyl, cyclo hexanol and secondary octyl phenyl are representative. Isobutyl, 2-ethyl hexyl sebacate is an example of a mixed ester. These esters may contain additional constituents or functional groups such as Cl, Br, NH<sub>2</sub>, NHR, NR<sub>2</sub>, CHO, CO, SH, SR, RSSR, ROR, ROMetal. The esters may be made by any of the methods for producing esters known to the art.

A suitable low temperature grease composition 20 may comprise di-2-ethyl hexyl sebacate and di-secondary butyl sebacate; with from 6 to 30% of a soap of a metal selected from the group consisting of alkali and alkaline earth metals together with a stabilizer consisting of an amphoteric metal compound, specifically an oxide carbonate or soap of zinc or aluminum. As further examples, the composition may consist of a major proportion, for example 65% or more, of di-secondary butyl adipate and di-isopropyl sebacate with 6 to 30% of soap and stabilizer as recited above.

One suitable method consists of reacting the alcohol with the acid at elevated temperatures in the presence of an esterification catalyst such as 35 sulfuric acid, sulfosalicylic acid, etc. The reaction is facilitated by a continuous removal of water formed during the reaction by azeotropic distillation with a solvent such as benzene, toluene, etc. or by passing inert gas through the reaction mixture to remove water of reaction. The product is washed with dilute alkali to remove the catalyst and any traces of unreacted acid and if necessary is heated under reduced pressure with or without blowing with an inert gas to remove 40 any unreacted alcohol or other low boiling material. If necessary the product can be clay-treated, and it is desirable although not absolutely necessary, that the finished ester have a neutralization number not higher than about 45 0.2 mg. KOH per gram of ester to obtain suitable stability to oxidation, since free acids left in the finished material can catalyze oxidation of the product, particularly in the presence of materials such as copper or brass at elevated temperatures.

50 Typical esters together with some of their more

3 significant properties are given in the following table.

4 completely melted. The grease was then rapidly cooled by running it over a drum chiller. It is

TABLE I

| Name of Ester                           | Centistokes Viscosity at— |         |           | Slope on ASTM Viscosity-Temp. Chart for the Interval of 210° F. to 40° F. | Visc. Index | Flash Point | Pour Point, ° F. | Appr. Boiling Point, ° F. At Atmospheric Pressure |
|-----------------------------------------|---------------------------|---------|-----------|---------------------------------------------------------------------------|-------------|-------------|------------------|---------------------------------------------------|
|                                         | 210° F.                   | 100° F. | —40° F.   |                                                                           |             |             |                  |                                                   |
| Di Sec. Butyl Sebacate.....             | 2.00                      | 6.42    | 320       | 0.752                                                                     | 136         | 255         | -90              | 650                                               |
| Di-2-ethylhexyl Sebacate.....           | 3.31                      | 12.64   | 1522      | 0.707                                                                     | 152         | 430         | -90              | 760                                               |
| Di-undecanyl Sebacate.....              | 4.66                      | 22.83   | 8000      | 0.716                                                                     | 138.5       | —           | -85              | —                                                 |
| D-2-ethylhexyl alkylated Succinate..... | 5.56                      | 42.72   | 1,200,000 | 0.812                                                                     | 68.5        | —           | -45              | —                                                 |
| Di-2-ethylhexyl Acetate.....            | 3.05                      | 11.26   | 1200      | 0.729                                                                     | 147         | 410         | -40              | 750                                               |

<sup>1</sup> Extrapolated from the 100 and 210° F. values.

It is readily apparent from the foregoing data that esters of this type possess ideal properties with regard to pour point, viscosity and viscosity-temperature characteristics, flash and boiling points necessary to minimize evaporation, making valuable lubricants for use as low temperature greases.

In making the greases of the present invention it is preferred to make the soap first, as for instance tallow, stearic acid or hydrogenated fish oil acids are reacted with alkali until an indicator shows the alkali to be present in slight excess. The soap thus formed is dried and if desired it may be powdered to facilitate solution in the ester. On the other hand the soap may in case of lithium, calcium, magnesium, or aluminum be prepared by precipitation from water by procedures well established in the art. The required amount of soap is then added to the ester and the mixture heated to from 360-400° F. until the soap is completely melted in the ester. Any of the alkalis or alkaline earth metals such as sodium or calcium, magnesium, strontium, lithium being preferred, may be used for neutralizing or saponifying the soap stock. As for the soap stock, any of the ordinary higher fatty acids or the fats from which they are derived such as stearic acid, oleic, erucic, lauric, palmitic acid, tallow, lard oil, animal fats, etc., although it is preferred to use the acid derived from hydrogenated fish oil, may be used to form the soaps with which to make the grease. On formulating the greases of the present invention they will contain in general alkali or alkaline earth soaps ranging from 6-30% of the total composition, 65-93.5% of the ester or mixture of several esters, and .5-5% of a stabilizer. The use of a stabilizer smooths out the texture of the grease and further aids in the actual production of the grease. The oxides, carbonates, or soaps of metals forming amphoteric oxides such as the soaps of zinc, tin and aluminum, have been found to be very beneficial in their use as stabilizers, particularly in the case of greases containing free alkali. Mixtures of these soaps may also be used, a particularly effective combination being .5% aluminum stearate and .5% zinc naphthenate.

The following specific example will serve to illustrate the invention in more detail.

*Example*

Per cent  
Lithium soap of hydrogenated fish oil acid... 12.0  
Aluminum stearate..... .5  
Zinc naphthenate..... .5  
2-ethylhexyl sebacate..... 87.0

The soaps and the esters were mixed together and heated to 360-400° F. until the soap had

20 permissible to allow the grease to cool in the equipment without working or to pour the molten grease into shallow pans to cool. The grease was then worked to the desired penetration or consistency, filtered and packaged.

25 For the purpose of comparing the greases of the present invention with low temperature greases of the prior art AN-G-3A Cone evaporation; bearing bleeding-oil leakage from lubricated anti-friction bearings and evaporation and plasticity number tests on representative samples were run with the following results:

TABLE II  
Bleeding and evaporation tests at 180° F.

| 35 | Lubricants | Cone Evaporation | 204-Ball Bearing Conrad Type |             |
|----|------------|------------------|------------------------------|-------------|
|    |            |                  | Bleeding                     | Evaporation |
|    |            |                  | Per cent                     | Per cent    |
| 40 | (1).....   | 7                | 0                            | .3          |
|    | (2).....   | 36.5             | —                            | —           |
|    | (3).....   | 8.3              | 0                            | .7          |
|    | (4).....   | 0.4              | 0                            | .05         |
|    | (5).....   | 0.2              | 0                            | .006        |

45 It will be noted that the usual type low temperature greases in use today are represented by grease 1. Thus around -70° F. the drag on the bearing is excessive. Greases 2 and 3 while having excellent low temperature properties are not 50 desirable due to their excessive rate of evaporation of the low boiling constituents in the greases. For example a bearing lubricated with grease 2 or 3 may be subjected to ground temperatures of 55 120 to 150° F. Due to excessive evaporation, the grease left in these bearings may not again be a suitable low temperature lubricant. Grease represented by Examples 4 and 5 have excellent 60 low temperature properties and also due to the high boiling esters used in their preparation are exceptionally stable at extremely high ground temperatures.

TABLE III  
Plasticity number (gram cm. seconds)

| 65 | Lubricants | -40° F. | -50° F. | -60° F. | -70° F. | -80° F. | -90° F. |
|----|------------|---------|---------|---------|---------|---------|---------|
|    |            | 8,000   | 10,000  | 15,000  | 20,000  | 30,600  | 1,000   |
|    | (1).....   | 8,000   | 10,000  | 15,000  | 20,000  | 30,600  | —       |
|    | (2).....   | —       | —       | 675     | 1,200   | 2,000   | 4,300   |
|    | (3).....   | —       | —       | —       | —       | —       | 10,000  |
|    | (4).....   | 625     | 825     | 1,100   | 1,500   | 2,200   | 3,300   |
| 70 | (5).....   | 1,400   | 2,200   | 2,900   | 3,800   | 5,000   | 8,000   |

Composition of the above greases

(1) Low your coastal oil (60 vis. at 100° F.; 300° F.) +12% soap.

## 5

- (2) Low pour coastal oil (35 vis. at 100° F.;/215° F.)+6% soap.  
 (3) Blend of low pour coastal oil and gas oil (45.2 vis. at 100° F.;/245) +12% soap.  
 (4) Secondary butyl sebacate, 12% lithium soap+1% stabilizer.  
 (5) 2-Ethylhexyl sebacate, 12% lithium soap+1% stabilizer.

From the above data it will be noted that the greases of the present invention are much superior to ordinary low temperature greases with respect to evaporation in both the cone and bearing evaporation tests and as stable against bleeding as the other greases. In the plasticity number test, numbers up to and including 2000 are in the free spinning range; from 2000-10,000 representing free turning and above 10,000 excessive torque or drag.

What is claimed is:

1. A low temperature grease consisting essentially of a major proportion of one or more compounds having the formula



where R is a bivalent aliphatic hydrocarbon radical; R<sub>1</sub> and R<sub>2</sub> are branched chain hydrocarbon radicals; a minor proportion comprising not more than 30% of a soap of a metal selected from the group consisting of alkali and alkaline earth metal and 0.5 to 5% of an amphoteric metal soap as a stabilizer.

2. A low temperature grease according to claim 1 in which R is a polymethylene radical having 8 methylene groups.

3. A low temperature grease composition according to claim 1 in which R<sub>1</sub> and R<sub>2</sub> are 2-ethylhexyl radicals.

4. A low temperature grease composition according to claim 1 in which R is a polymethylene radical having 8 methylene groups and R<sub>1</sub> and R<sub>2</sub> are secondary butyl radicals.

5. A low temperature grease comprising at least 65% of a compound having the formula



where R is a bivalent aliphatic hydrocarbon radical; R<sub>1</sub> and R<sub>2</sub> are branched chain hydro-

## 6

carbon radicals; 6-30% of a soap of a metal selected from the group consisting of alkali and alkaline earth metal and 0.5 to 5% of an amphoteric metal soap as a stabilizer.

6. A low temperature grease comprising at least 65% of a compound having the formula



where R is a bivalent aliphatic hydrocarbon radical; R<sub>1</sub> and R<sub>2</sub> are branched chain hydrocarbon radicals; 12% of a soap of a metal selected from the group consisting of alkali and alkaline earth metal and 1% of a compound selected from the class consisting of the oxides, carbonates and soaps of amphoteric metals as a stabilizer.

7. A low temperature grease according to claim 1 in which the soap of a metal is 6-30% of lithium soap of hydrogenated fish oil acids.

8. A low temperature grease composition comprising at least 65% of di-2-ethylhexyl sebacate; 6-30% of a soap of a metal selected from the group consisting of alkali and alkaline earth metal and 0.1 to 5% of an amphoteric metal soap as a stabilizer.

9. A low temperature grease composition comprising at least 65% of the ester isobutyl, 2-ethylhexyl sebacate; 6-30% of a soap of a metal selected from the group consisting of alkali and alkaline earth metal and 0.5 to 5% of an amphoteric metal soap as a stabilizer.

JOHN C. ZIMMER.

ARNOLD J. MORWAY.

## REFERENCES CITED

- 35 The following references are of record in the file of this patent:

## UNITED STATES PATENTS

| Number       | Name              | Date          |
|--------------|-------------------|---------------|
| 40 1,993,738 | Graves            | Mar. 12, 1935 |
| 2,104,408    | Wiezevich         | Jan. 4, 1938  |
| 2,134,736    | Reuter            | Nov. 1, 1938  |
| 2,158,096    | Werntz            | May 16, 1939  |
| 2,204,601    | Kavanagh et al.   | June 18, 1940 |
| 45 2,351,280 | Morgan I          | June 13, 1944 |
| 2,362,767    | Morgan II         | Nov. 14, 1944 |
| 2,363,513    | Farrington et al. | Nov. 28, 1944 |